

## UNITED STATES PATENT OFFICE

2,050,646

LINOLEUM AND METHOD OF  
MANUFACTURING

Robert D. Bonney, Glen Ridge, and Walter S. Egge, West Orange, N. J., assignors to Con-goleum-Nairn Inc., a corporation of New York

No Drawing. Application June 30, 1934,  
Serial No. 733,305

24 Claims.

(Cl. 18—55)

The present invention relates to the manufacture of mouldable compositions having a binder obtained from oxidized oil, said compositions including particularly linoleum and similar articles, and more especially to an improved process of manufacturing such compositions and to the improved products resulting from such process.

Various types of compositions, generically termed "linoleum" were developed and patented (United States Patent No. 87,277) by Frederick Walton over sixty years ago. His original linoleum compositions included oxidized and solidified linseed oil, rosin, and kauri gum, specially prepared and fluxed together to form a binder or cement, this binder being then combined with pigments, wood flour, ground cork, and mineral fillers. It is characteristic of the compositions that they are plastic when freshly prepared and warm so that they may be rolled or pressed into sheet form and subsequently or simultaneously united with a backing or supporting sheet and that, subsequent to forming into the desired shape, they may be cured or seasoned by long continued exposure to heated air to the elastic firmness characteristic of the finished product.

While many changes have since been made in the proportions of the materials used in linoleum compositions, and various additions and substitutions have been proposed, sometimes with a view to decreasing the proportion of linseed oil and other costly constituents, and sometimes with a view to improving some quality of the product, the essential components of linoleum, its structure and physical characteristics, and even the methods and equipment for producing it are today generically the same as they were sixty years ago. Particularly is this true of the oxidized oil-resin-gum binder and it is to a major change in the character and composition of this component that our invention is primarily directed.

The linoleum binder is commonly called a "cement" by those skilled in the art. According to prior practice, all linoleum cements comprise an oxidized and solidified drying or semi-drying oil, usually linseed oil, intimately fluxed with resinous material, usually rosin. There are two general methods employed today for producing such cements. The older is the two-stage method involving: (a) the oxidation and solidification of the linseed oil; and (b) the refluxing of the solidified oil with resins and gums. The first step (a) may be accomplished by either of two conventional methods: one, the Walton or "scrim" process; and the other, the Wood-Bedford or mechanically oxidized oil process. The Walton process (British Patent No. 209 of 1860) consists in successively flooding vertically suspended cotton fabrics, called "scrims", with linseed oil which has been boiled with suitable driers,

each layer of oil being allowed to oxidize and coagulate or solidify before being followed by the next flooding. The process is exceedingly slow, requiring from two to four months to produce a "skin" of oxidized and solidified oil suitable for use. The Wood-Bedford method (British Patent No. 7,742 of 1893) on the other hand, is a rapid process, being completed in twelve to eighteen hours. It consists essentially in aerating and agitating the linseed oil, together with suitable driers, in a closed cylindrical vessel at a temperature of approximately 180° F., the aeration and agitation being continued until the oil is oxidized and solidified to the desired consistency. The Wood-Bedford method offers a great advantage in time saving, but unfortunately the solidified oil produced thereby is usually somewhat inferior to that produced by the "scrim" process. The second step (b) in the two-stage method is the original, yet up-to-date, process described by Walton and consists in fluxing, in a kettle of well known construction, the solidified oil, produced in the first stage, with resinous material such as rosin, kauri gum, etc. The oxidized and solidified oil produced by either the Walton or Wood-Bedford method above described may be used, but in order to produce a wholly satisfactory cement it has usually been found necessary to use at least a substantial amount of the Walton or "scrim" process oil. The proportion of resinous material may vary from 20% to 35%, by weight, but generally such resinous material comprises a considerable proportion of rosin. The fluxing is carried on at a temperature of 250° to 340° F. and under conditions substantially excluding air. The solidified oil, upon agitation with the rosin constituent of the resinous material, becomes somewhat mobile and in this state the several constituents of the cement may be thoroughly and intimately mixed. Upon continued heating, however, the viscous mix commences to resolidify and such resolidification is permitted to proceed until the mass is adjudged by the operator to be of the proper consistency for cement. It is then dumped into pans to cool.

The second method currently used for preparing linoleum cement is the single stage process developed by Ingle (British Patent No. 1,021 of 1910). According to this method approximately three parts of linseed or other drying or semi-drying oil, or mixtures thereof, and one part of rosin or equivalent resinous material are placed in an oxidizer of the Wood-Bedford type, the mix heated to a temperature of about 180° F. and aerated with constant agitation for a period of 14 to 24 hours. During the treatment the oil becomes oxidized and partially solidified, the process being stopped and the mass dumped when the desired consistency for a good cement is obtained.

It is a fundamental characteristic of these pre-

5

10

15

20

25

30

35

40

45

50

55

60

vious methods of manufacturing linoleum cement that the oxidized oil from which the cement is prepared contains a substantial or major proportion of coagulated constituents (i. e. linoxyn) 5 and is substantially or essentially solid at sometime before the preparation of the cement is completed. One method of chemically evaluating linoleum and linoleum cements consists in separating oxidized and solidified oil or cement into 10 three components, namely, Fraction I, that component which is coagulated and is insoluble in ethyl ether and which is known as linoxyn and comprises coagulated oxidized glycerides of linolic and linolenic acids; Fraction II, that component 15 soluble in ethyl ether but insoluble in petroleum ether, comprising chiefly the oxidized but uncoagulated linolic and linolenic glycerides of the drying oil and capable of hardening without further substantial oxidation; and Fraction III, 20 that component soluble in petroleum ether, comprising chiefly the unoxidized and non-hardening constituents of the oxidized drying oil, including unoxidized glycerides of linolic and linolenic acids, unoxidizable and non-hardening glycerides 25 of saturated fatty acids, and oxidized but non-hardening glycerides such as oxidized glycerides of oleic acid. The term "non-hardening" is employed herein to indicate the property of retaining fluidity, even under the action of air, for 30 long periods.

It is a fundamental characteristic of all linoleum cements heretofore produced or known that each comprises not only linoxyn but also all other constituents of the oxidized oil in substantially the 35 proportions in which they naturally occur in the oxidized oil. Thus, it is a fundamental characteristic of all the linoleum cements heretofore produced or known that each comprises a substantial proportion of linoxyn, i. e., Fraction I. 40 On the basis of the total oil content of the cement, the percentage of linoxyn may vary from 30% to 55%, by weight. Similarly, it is characteristic of all linoleum cements heretofore produced or known that each comprises a substantial percentage of unoxidized and non-hardening constituents of the oxidized oil, i. e., Fraction III. These constituents of Fraction III may vary from 15% to 40%, by weight, on the 45 basis of the total oil component of the cement. 50 As a result, the proportion of the oxidized but uncoagulated glycerides of linolic and linolenic acids, i. e., Fraction II, will vary from 25% to 45% by weight. The definite and substantial proportion of linoxyn present in all linoleum cements is 55 required to offset or overcome the fluidity imparted to the cement by the presence of the likewise substantial amount of unoxidized and non-hardening oil constituents of the oxidized oil, thus providing rigidity and toughness in the cement structure in spite of its substantial content 60 of fluid non-hardening constituents. As a corollary the substantial proportion of fluid non-hardening constituents in the cement requires the presence of a substantial or major proportion of 65 coagulated constituents to produce an effective and practicable cement. Such function of the linoxyn is believed to be accomplished by occlusion of the constituents of Fraction III in the coagulated molecules of the linoxyn which, 70 through association, assume colloidal dimensions. Whether or not this is the correct theory, the fact remains that to produce a satisfactory finished linoleum, it has always been found necessary to prepare the cement binder in the form of a tough, 75 rubbery, elastic-solid, requiring very heavy ma-

chinery to handle and characterized by its poor or slow wetting properties.

Our invention is based upon discoveries regarding the effect of varying the composition and mode of preparation of the oxidized oil component of the cement. Thus we have found that if a substantial proportion of the un- 5 oxidized and non-hardening constituents normally present in the oil base of the cement, i. e., Fraction III, are eliminated, a linoleum cement 10 of remarkable physical and chemical properties can be produced. Also, we have found that, coincident with such reduction in the proportion of these constituents, a highly satisfactory linoleum cement possessing unexpected advantages 15 can be prepared which is in fluid phase, by causing the cement to be substantially devoid of any linoxyn content or to possess a substantially decreased ratio of linoxyn to those fluid constituents of the oxidized oil which are capable 20 of hardening without further substantial oxidation. Such a modified cement, when admixed in the usual proportion with the common filler and pigment materials, forms a linoleum composition that may be properly seasoned or cured 25 in a fraction of the usual period and which, when seasoned, produces a finished linoleum having highly improved properties as hereinafter more fully described. Furthermore, such linoleum cement, being prepared in fluid phase rather than 30 as an elastic-solid, may be incorporated with the filler materials more thoroughly and in less time because of its high wetting properties and with but a fraction of the usual power requirements.

One embodiment of the process of our invention in the manufacture of the improved linoleum or other mouldable compositions constituting the product of our invention comprises the steps of subjecting a substance which contains a drying or semi-drying oil, and which may contain 35 a resinous material, to an oxidizing treatment limited substantially to the formation of uncoagulated products of the oxidation, treating the oil to remove therefrom a substantial proportion of unoxidized and non-hardening oil constituents, admixing the so prepared component of oxidized oil with filler materials to form a mouldable composition, moulding the mix by pressure, and effecting partial conversion of constituents 40 of the oxidized oil component into linoxyn, there- 45 by producing a sufficiently cured product, the effecting of such conversion being divided between the mixing, moulding, and curing steps in 50 such proportion as desired. Our product invention contemplates a finished linoleum or other 55 composition of unusual flexibility and resistance to moisture and soiling, comprising a binder in which the oil component is characterized by a substantially reduced ratio of unoxidized and 60 non-hardening oil constituents to all other constituents of the oil component as compared with the ratio characterizing oil binders of linoleum heretofore known.

In preparing the improved linoleum of our invention, we prefer to employ linseed oil as the 65 oil base for the modified cement. Other drying or semi-drying oils such as perilla oil, rubberseed oil, or soya bean oil may be used, and in general any drying or semi-drying oil which, upon oxidation, yields a substantial amount of 70 the oxidized glycerides of linolic and/or linolenic acids in fluid phase will be found satisfactory. Also the modified cement of our improved linoleum should contain a substantial proportion of resinous material. A wide choice 75

of suitable resinous materials is available, among which may be mentioned rosin, ester gum, fused congo, congo ester, kauri gum, paracoumarone resin, oil-soluble or oil-reactive synthetic resins 5 of the phenol-aldehyde type, either with or without rosin, etc. For ordinary purposes wood rosin will be found most desirable since it is inexpensive, uniform in quality, and easily soluble in the oil. For special purposes, or to obtain special 10 properties in the finished linoleum, other resins may prove more satisfactory. It will be found preferable to incorporate such resinous material with the oil base prior to the oxidation treatment. The presence of resin not only facilitates 15 the oxidation of the oil but markedly improves the toughness of the final linoleum product. Also by such procedure it becomes possible to incorporate with the oil component certain resins which could not otherwise be incorporated such 20 as paracoumarone, and certain glyptals, amberol, and bakelite resins having a relatively low acid value. It should be pointed out that it is not necessary to incorporate the selected resinous material with the oil base prior to oxidation, 25 as good results may also be obtained by first preparing the oxidized and treated oil in the manner hereinafter described and then adding thereto, preferably in solution, the selected resin.

By way of illustrating the various aspects of 30 our process invention, we will describe in detail a preferred embodiment thereof. Three parts of linseed oil and one part of wood rosin, by weight, are heated in a Wood-Bedford type of oxidizer to about 240° F. until the resin is dissolved. The temperature is then lowered to 35 about 180° F. and a suitable drier, for example, .04% cobalt linoleate, is added. The batch, at a temperature of approximately 180° F., is then blown with air or equivalent oxygen-containing 40 gas for a period of 20 to 30 hours. When a tested sample just fails to completely dissolve in ethyl ether, the oxidation is discontinued. The batch is then cooled and treated to effect a separation of the unoxidized and non-hardening 45 constituents from the desired oxidized oil constituents. This separation may be effected by subjecting the oxidized oil or oil-resin mix to selective extraction with a solvent capable of dissolving the undesirable constituents but possessing 50 little if any solvating action upon the oxidized but uncoagulated constituents which are desirable for our improved linoleum cement and which are fluid and are capable of hardening without further substantial oxidation. The preferred solvent is petroleum ether (boiling range 55 30° to 75° C.), and about 3 to 4 volumes thereof to 1 volume of the oxidized oil or oil-resin mix should be employed. Petroleum naphtha (boiling range 60° to 160° C.) may be used as an 60 equivalent extracting solvent. Those oxidized but uncoagulated constituents of the oil or oil-resin mixture which are desirable constituents for the linoleum cement, and a major portion of the resinous material, form a lower layer, while substantial proportions of the unoxidized and non-hardening oil constituents dissolve in the extracting solvent forming an upper layer. This upper layer is removed by decantation. The extraction process is preferably repeated two or 65 three times to assure an adequate separation. The remaining portion of the oxidized oil or oil-resin mix, in fluid phase, is then subjected to low heat, and preferably at reduced pressure, to remove the last portion of the extracting solvent, 70 after which it is ready for use as or in our im-

proved linoleum cement. For convenience in handling, and to prevent premature solidification or gelation, the desired constituents of the oxidized oil or oil-resin mix, in fluid phase, obtained by the oxidizing and separating treatment above described, are preferably dissolved in a suitable solvent such as toluol, butyl acetate, xylene, high-flash coal tar naphtha, etc., to provide a 60 to 80% solution. Where the resinous material is incorporated with the oil component prior to the 10 oxidation treatment, this solution of the desired constituents of the oxidized and treated oil-resin mix constitutes the cement for our improved linoleum. Where the resinous material is not incorporated with the oil base prior to the oxidizing treatment, the oxidation of the oil alone and the separation of the undesirable from the desirable constituents of the oxidized products will be carried out in the same manner as above described and to the solution of the separated desired constituents of the oxidized oil may be added the selected resinous material. In either case, it will be found preferable to formulate the cement so that the non-volatile component thereof will comprise approximately one part of resinous 25 material to three parts of the desired oxidized and separated oil constituents in fluid phase. However, the addition of the resinous material is not critical to the realization of many of the advantages of our invention, and it is within the 30 purview of the invention to omit the resinous material and to employ solely the prepared oil component in formulating the modified and improved cement, particularly where a softer composition may be desired. 35

It is to be noted that in the treatment of the raw oil or oil-resin mix to produce the cement, the oxidation is discontinued at, or just before the point where constituents of the oxidized oil have commenced to coagulate to the gel or linoxyn phase. This point may be determined by the ethyl ether test. So long as no linoxyn is formed, the constituents of the batch undergoing oxidation will dissolve completely in ethyl ether, but upon the formation of linoxyn, a cloud-like 40 precipitate will appear in the sample tested. Following the above described method, the yield of oxidized but uncoagulated constituents of the oil which are in fluid phase and are desirable ingredients of the linoleum cement, i. e., that portion 45 of the oxidized oil soluble in ethyl ether, but insoluble in petroleum ether, varies from 60 to 75% by weight of the oil after completion of the oxidizing treatment thereof. To a considerable extent the yield depends upon the nature of the 50 resin employed. A resin such as rosin, which is strongly acid in character, serves apparently as a peptizing agent to retard the coagulation of the oxidized constituents of the oil, thus increasing the yield of these desired oxidized constituents in fluid phase. On the other hand, if no resin is employed or if a nearly neutral resin is selected, the yield will be lower. When employing no resin, or a neutral or weakly acid resin, in the preparation of the oil component of the 55 cement, the percentage yield of the desired oxidized constituents of the oil may be somewhat increased by adding to the oil or oil-resin mix prior to oxidation a small amount—1% to 2.0%—of maleic acid (maleic acid anhydride) or 60 equivalent acidic substance, difficultly volatile at the processing temperature. The maleic acid or maleic acid anhydride may be added in dry state but is more conveniently added in the form of an acetone solution. 65 70 75

- 5 The desired oxidized oil constituents of the modified cement, which are soluble in ethyl ether but insoluble in petroleum ether, comprise chiefly the oxidized glycerides of linolic and linolenic acids in fluid phase and uncoagulated. These constituents have the property of coagulating or hardening by conversion into linoxyn without substantial further oxidation and even without contact with air. The unoxidized constituents 10 of the oil which are not oxidized in the oxidizing treatment, which is so conducted as to produce the desired oxidized constituents in fluid phase, are either constituents of the oil which cannot be oxidized by such treatment or by contact with 15 air and do not possess the property of hardening such as the glycerides of saturated organic acids of which stearic or palmitic are examples, or they are constituents of the oil which are capable of being converted by the oxidizing treatment into 20 substances having the property of hardening, but were not so converted, such as the glycerides of linolic and linolenic acids. The other products of the oxidizing treatment which are undesirable as constituents of the modified cement, are those 25 oxidized oil constituents which do not possess the property of coagulating even though oxidized such as the oxidized glycerides of oleic acid. It is these unoxidized and non-hardening constituents of the oil normally present after completion 30 of the oxidizing treatment which are removed to a substantial extent by the separation treatment above described.
- 35 Although it is desirable that the amount of unoxidized and non-hardening oil constituents, remaining in the linoleum cement as prepared, should be at a minimum, nevertheless the difficulty and expense of securing in commercial operation a quantitative elimination of these constituents, makes it inexpedient to attempt to obtain this end. As above pointed out, the 40 advantages of this invention accrue from the elimination from the linoleum cement of a substantial proportion of the unoxidized and non-hardening oil constituents of the oxidized drying or semi-drying oil base, thus making possible the preparation 45 of an improved cement in fluid phase which contains little or no linoxyn. This aim may be accomplished when the separation of the desirable and undesirable constituents of the oxidized oil is carried to such an extent that the oil component of the cement contains approximately 93% or more of oxidized but uncoagulated oil constituents soluble in ethyl ether but insoluble in petroleum ether. Defining in another way the 50 chemical character of the modified cement for producing our improved linoleum, the advantages of our invention may be realized if, in such cement, the ratio of the unoxidized and non-hardening oil constituents, to all other oil constituents of the cement, is 1 to 12 or more. By way of comparison, the corresponding ratio of these constituents in the conventional type of commercial linoleum cements heretofore known is almost invariably 1 to 6 or less.
- 55 The next step in our improved process of manufacturing the products of our invention is to combine with the modified cement prepared as above described, the requisite filler materials to form a mouldable composition. Normally the 60 improved linoleum will comprise a proportion of vegetable fillers such as ground cork or wood flour and a proportion of mineral fillers such as whiting, china clay, asbestos, etc., as well as pigments including both white pigments and the desired coloring pigments. The particular fillers

and pigments and the proportions in which they may be employed are not essential features of our invention. In general we propose to employ any of the vegetable and mineral fillers which have been heretofore known or used in linoleum 5 compositions and we propose to employ such fillers in the amounts and proportions recognized as standard practice. A generic formula may be stated as follows:—

|                                    |            |    |
|------------------------------------|------------|----|
| Modified cement                    | 25% to 50% | 10 |
| Vegetable fillers                  | 25% to 35% |    |
| Mineral fillers including pigments | 25% to 40% |    |

Depending upon the nature of the product desired, however, the proportion of the vegetable 15 filler may be increased above or decreased below the limits specified with a corresponding decrease or increase in the proportion of mineral fillers and pigments or one type of filler may be used to the exclusion of the other type. 20

A typical example, illustrating the formulation of our improved linoleum is as follows:—350 pounds of an 80% solution (in hi-flash naphtha) of the oxidized and treated oil-resin cement prepared as above described is admixed with 300 25 pounds of wood flour in a conventional type of Pfleiderer mixer, the mixer being warmed to drive off the solvent. After a preliminary mixing of the improved cement and wood flour, 200 pounds of whiting and 200 pounds of lithopone 30 are then added and the mixing is continued until the mass becomes thoroughly homogeneous and yields a smooth, strong sheet when calendered. The temperature of the mix should usually be regulated so as not to exceed approximately 180° 35 F. and preferably the mixing should be carried out, at least during its early stages, at substantially lower temperatures. The period of mixing will be determined by the type of linoleum to be made. Thus, composition to be pressed 40 or calendered directly onto a burlap or other base web, as in the production of either the so-called moulded inlaid or the plain linoleum, need be mixed only a few minutes whereas composition to be formed into unbacked sheets for cutting 45 and inlaying will be mixed for a longer period in order that the freshly calendered sheet produced therefrom may be tougher. The homogenized mix of fillers and cement is dumped from the mixer and disintegrated in any conventional manner as by passing it through a "german" or "scratcher" or both, after which it is 50 ready for sheeting in accordance with standard practice.

One marked advantage of our invention is the 55 ease with which the mouldable composition may be prepared. Since the cement is incorporated while in fluid phase, good wetting and dispersion thereof are facilitated and much lighter mixing machinery may be used. The total time required 60 for thoroughly mixing the several ingredients is reduced by 50% or more. Most important of all, the power required for effecting the mixing of the fillers and binder may be as little as 10% of that normally required by the conventional methods 65 now employed where the linoleum cement is prepared and used in the form of a tough, rubbery elastic-solid. As above indicated, the temperature at which the mixing operation is conducted and the period over which it is extended may 70 vary in accordance with the character of the linoleum composition desired. Higher temperatures, i. e., temperatures of the order of 180° F., and longer mixing periods will effect a limited conversion into linoxyn of the oxidized but fluid 75

constituents of the oil component of the binder and the more extensive the formation of linoxyn in this mixing stage, the tougher will be the resulting composition when calendered or sheeted.

5 In general limited formation of linoxyn during the mixing operation is desirable, but to facilitate thorough dispersion of the binder and to effect incorporation of the fillers with a minimum expenditure of power, such formation of linoxyn 10 should be restricted during the early stages of the mixing. This regulation may be readily accomplished by control of the temperature of the mix, lower temperatures being preferably employed during the early stages of the mixing 15 operation and higher temperatures being permitted only after thorough dispersion of the fluid cement whereby the formation of any substantial proportion of linoxyn occurs only near the end of the mixing operation.

20 The linoleum composition prepared as above described and sheeted, calendered, or otherwise moulded by pressure into the desired form is finally subjected to a seasoning treatment to effect a further conversion or solidification of the 25 oxidized but uncoagulated oil constituents of the binder into linoxyn. This seasoning or curing is preferably carried out at elevated temperatures, two to four days being required at a temperature of 170° F. Linoleum of our invention may however be seasoned at lower temperatures or at temperatures as high as 200 to 210° F. in which latter case the seasoning period will be shortened to about 24 hours. By way of contrast, linoleum composition prepared according to the process 30 heretofore known and used, requires a seasoning period varying from 7 to 40 days at a temperature of 170 to 180° F. and in the heavier gauges cannot successfully be seasoned above this temperature without formation of a so-called "wet seam", that 35 is, a sheet having a hard surface and a soft center. The importance of this substantial reduction in seasoning period will be apparent to those skilled in the art.

The improved linoleum of our invention resulting from the process just described is characterized by markedly improved flexibility, such superior flexibility being present not only when the linoleum is freshly manufactured but continuing indefinitely as the product ages. This 40 characteristic is attributable to the substantial reduction in the proportion of the unoxidized and non-hardening constituents of the oil component of the cement which constituents have no binding power in themselves but when present 45 are strongly adsorbed into the capillary structure of the linoxyn formed during the seasoning treatment and subsequent aging so that such linoxyn behaves like a rigid solid. Our improved linoleum also exhibits substantially increased resistance to soiling and to moisture. This is attributable to the very thorough wetting of each 50 particle of the vegetable filler material obtainable by incorporating the oxidized oil binder in the form of a fluid instead of an elastic-solid. The 55 particles of vegetable filler thus become impregnated and coated with the cement and are thereby rendered highly water-resistant. Furthermore, as will be noted in the description of the process, the mineral fillers and pigments are 60 preferably added after the vegetable fillers have been pre-mixed with the cement, this sequence of operations permitting each particle of the vegetable filler first to be covered with cement and such cement-covered particles then to become 65 coated with mineral fillers thereby greatly

improving the resistance of the linoleum to soiling or traffic while preserving the resiliency for which linoleum as a product is renowned.

According to the conventional method, above referred to, of chemically evaluating linoleum and linoleum cements, our improved linoleum product is characterized by a substantially decreased ratio of unoxidized and non-hardening constituents (i. e., Fraction III) of the oxidized oil component of the binder to those oil constituents of the binder present in the form of linoxyn and in the form of oxidized but uncoagulated products of oxidation. In linoleum prepared according to conventional processes heretofore known or used, about 20% of the unoxidized constituents 10 of the oil component of the cement are converted into oxidized or oxidized and coagulated constituents during the seasoning treatment. This conversion also continues, though at a slow rate, as the linoleum ages. Thus, as compared with 20 the 15% to 40% of unoxidized and non-hardening constituents (i. e., Fraction III) normally present in the oil component of the conventional type of linoleum cement before seasoning, the percentage in such linoleum cement may be reduced to 12% to 30% after seasoning of the linoleum and 10% to 25% after years of aging. Expressed in another way the ratio of these constituents to the remainder of the constituents 25 of the oil component of the binder of conventional linoleum is normally at least 1 to 7 after seasoning and normally at least 1 to 9 even after long aging. In contrast to these percentages and ratios, our improved linoleum after the seasoning treatment comprises a binder or cement 30 wherein the unoxidized and non-hardening constituents of the oil component, i. e.—constituents soluble in petroleum ether—are but approximately 6% or less of the total oil component of the cement and the ratio of such undesirable 35 constituents to the remainder of the constituents of the oil component is less than 1 to 15, normally about 1 to 20.

It will be apparent to those skilled in the art that this invention constitutes a major advance 45 in the linoleum industry. It will also be clear that the teachings of the improved composition or linoleum product and of the various steps in the method of producing such composition or product as set forth herein may be applied in 50 many ways to secure one or more of the enumerated or recognized advantages, or may be modified in different aspects without departing from the spirit of the invention. Thus, for example, the improved binder or cement of our invention 55 may be employed in conjunction with other binders, as, for example, nitrocellulose, chlorinated rubber, or the like in preparing mouldable compositions or cements therefrom, such composite cements or binders possessing those advantages 60 accruing from the presence therein of an oil component prepared in accordance with our invention. The several features of this invention co-operate in such manner, when they are all used 65 in conjunction, as to produce results that are due to such cooperation and are additional to such results as flow from the separate use of those features or from a use of those features in such manner that they are not properly coordinated; and in the best practice of our invention, all of 70 the features above described, or equivalent features, will preferably be employed in the cooperative relation above described, or equivalent relation. However, certain of those features, such as the reduced content of non-hardening and 75

unoxidized constituents of the oxidized oil product to which fillers, etc., are added, and also the fluidity of the material to which fillers, etc., are added, used either singly or in the absence of 5 one or more of the several features described, produce novel and advantageous results when so used, and such use falls within the spirit of our invention. It is to these fundamental teachings as set forth in the foregoing specification herein 10 that the inventors assert their pioneer ship.

We claim:

1. The process which comprises the steps of subjecting a drying or semi-drying oil to an oxidizing treatment, discontinuing the oxidizing treatment prior to substantial coagulation of the oxidized oil, treating the products of oxidation to remove therefrom a substantial proportion of unoxidized oil constituents and non-hardening oil constituents, admixing filler material with the remaining fluid oxidized oil constituents to form a mouldable composition, moulding the mix by pressure, and subjecting the moulded mixture to treatment for converting oxidized oil constituents therein into linoxyn.
2. The process which comprises the steps of admixing a drying or semi-drying oil and resinous material, subjecting the mixture to an oxidizing treatment, discontinuing the oxidizing treatment prior to substantial coagulation of oxidized oil constituents to form linoxyn, treating the products of oxidation to remove therefrom a substantial proportion of the constituents of the oil which are unoxidized or non-hardening, admixing filler material with the remaining fluid oxidized oil-resin binder to form a mouldable composition, moulding the mix by pressure, and subjecting the moulded mixture to treatment for converting oxidized oil constituents therein into linoxyn.
3. The process which comprises the steps of subjecting a drying or semi-drying oil to an oxidizing treatment, discontinuing the oxidizing treatment prior to substantial coagulation of oxidized oil constituents to form linoxyn, treating the products of oxidation to remove therefrom a substantial proportion of the unoxidized oil constituents and non-hardening oil constituents, combining with the fluid oxidized oil constituents a resinous material, admixing filler material with the prepared oxidized oil-resin binder to form a mouldable composition, moulding the mix by pressure, and subjecting the moulded mixture to treatment for converting oxidized oil constituents therein into linoxyn.
4. The process which comprises the steps of subjecting a substance comprising a drying or semi-drying oil to an oxidizing treatment limited substantially to formation of uncoagulated products of oxidation, selectively extracting from the products of oxidation the unoxidized and non-hardening constituents of the oil, combining the remaining fluid oxidized constituents of the oil with filler material to form a mouldable composition, moulding the mix by pressure, and subjecting the moulded mixture to treatment for converting oxidized oil constituents therein into linoxyn.
5. The process which comprises the steps of subjecting a substance comprising a drying or semi-drying oil to an oxidizing treatment limited substantially to the formation of uncoagulated products of oxidation, selectively extracting the resulting product with a low boiling liquid hydro-carbon to remove unoxidized and non-hardening

oil constituents, admixing filler material with the remaining fluid oxidized oil constituents to form a mouldable composition, moulding the mix by pressure, and subjecting the moulded product to the action of an elevated temperature to effect 5 conversion of oxidized oil constituents into linoxyn.

6. The process which comprises the steps of subjecting a substance comprising a drying or semi-drying oil and an acidic resin to oxidizing 10 treatment limited substantially to the formation of uncoagulated products of oxidation, extracting the resulting product with low boiling liquid hydro-carbon to remove unoxidized and non-hardening oil constituents, admixing the remaining fluid oxidized oil constituents with filler material to form a mouldable composition, moulding the mix by pressure, and seasoning.

7. The process which comprises the steps of subjecting a substance comprising a drying or 20 semi-drying oil to oxidation treatment limited substantially to the formation of uncoagulated products of oxidation, treating the product to remove therefrom the unoxidized and non-hardening oil constituents, combining the fluid oxidized 25 oil constituents with 50% or more of vegetable and/or mineral fillers to form a mouldable composition, moulding the composition, and seasoning.

8. The process which comprises the steps of 30 subjecting a substance comprising a resinous material and a drying or semi-drying oil to an oxidizing treatment limited substantially to the formation of uncoagulated products of oxidation, treating the oxidation products to remove therefrom 35 a substantial proportion of the non-hardening constituents thereof, combining the remaining fluid oxidized oil-resin constituents with 50% or more of vegetable and/or mineral fillers to form a mouldable composition, moulding the composition into the desired form, and subjecting the moulded product to heat to convert oxidized oil constituents 40 therein into linoxyn.

9. The process which comprises the steps of subjecting a substance comprising a drying or 45 semi-drying oil to an oxidizing treatment limited substantially to the formation of uncoagulated products of oxidation, treating the product to remove therefrom unoxidized and non-hardening oil constituents, premixing the remaining fluid 50 oxidized oil constituents with a vegetable filler, adding mineral fillers to the premix to form a mouldable composition, moulding the composition by pressure, and effecting conversion of oxidized oil constituents 55 therein into linoxyn.

10. The process which comprises the steps of subjecting a substance comprising a resinous material and a drying or semi-drying oil to an oxidizing treatment limited substantially to the formation of uncoagulated products of oxidation, 60 treating the product to remove therefrom a substantial proportion of the non-hardening constituents thereof, premixing the remaining fluid oxidized oil-resin constituents with a vegetable filler, adding mineral fillers to the premix to form a mouldable composition, moulding the composition into the desired form, and effecting conversion of oxidized oil constituents 65 therein into linoxyn.

11. The process which comprises the steps of 70 subjecting a substance comprising a drying or semi-drying oil to an oxidizing treatment limited substantially to the formation of uncoagulated products of oxidation, separating the product into a fraction which is richer than said product in 75

fluid oxidized oil constituents, and capable of hardening without further substantial oxidation, and a fraction which is richer than said product in unoxidized and non-hardening oil constituents, 5 admixing filler material with the first named fraction to form a mouldable composition, moulding by pressure, and seasoning.

12. The process which comprises the steps of subjecting a substance comprising a resinous material and a drying or semi-drying oil to an oxidizing treatment limited substantially to the formation of uncoagulated products of oxidation, separating the product into a fraction which is richer than said product in fluid oxidized oil constituents, and capable of hardening without further substantial oxidation, and a fraction which is richer than said product in unoxidized and non-hardening oil constituents, admixing the first named fraction with filler material to form a mouldable composition, moulding by pressure, and seasoning.

13. In a process for producing a composition comprising constituents of oxidized drying or semi-drying oil, the steps comprising subjecting a drying or semi-drying oil to an oxidizing treatment, treating the products of oxidation to remove therefrom a substantial proportion of unoxidized oil constituents and non-hardening oil constituents, admixing filler material with the remaining fluid oxidized oil constituents to form a mouldable composition, moulding the mix by pressure, and subjecting the moulded mixture to treatment for converting oxidized oil constituents therein into linoxyn.

14. In a process for producing a composition comprising constituents of oxidized drying or semi-drying oil, the steps comprising subjecting a drying or semi-drying oil to an oxidizing treatment, discontinuing the oxidizing treatment prior to substantial coagulation of the oxidized oil, treating the products of oxidation to remove therefrom a substantial proportion of unoxidized oil constituents and non-hardening oil constituents, dissolving the remaining fluid oxidized oil constituents in a suitable solvent, admixing filler material with such solution to form a mouldable composition, and moulding said composition.

15. Linoleum or similar composition composed of filler material and a binder comprising the hardened component of oxidized drying or semi-drying oil which, after oxidation of the oil is in fluid phase, is separated from a substantial proportion of unoxidized and non-hardening oil constituents of the oxidized oil, and is capable of hardening without further substantial oxidation.

16. Linoleum or similar composition composed of filler material and a binder comprising a resinous substance and the hardened component of oxidized drying or semi-drying oil which, after oxidation of the oil is in fluid phase, is separated from a substantial proportion of unoxidized and non-hardening oil constituents of the oxidized oil, and is capable of hardening without further substantial oxidation.

17. Linoleum or similar composition composed of vegetable and/or mineral fillers and 25% to 50% of a binder comprising the hardened component of oxidized drying or semi-drying oil which, after oxidation of the oil is in fluid phase, is separated from a substantial proportion of non-hardening oil constituents of the oxidized oil, and is capable of hardening without further substantial oxidation.

18. A mouldable composition comprising filler material and a binder comprising the fluid com-

ponent of oxidized drying or semi-drying oil which is capable of hardening without further substantial oxidation, and is separated from a substantial proportion of unoxidized and non-hardening oil constituents of the oxidized oil, and sufficient solvent for said fluid component to maintain its fluidity. 5

19. A mouldable composition comprising filler material and a binder comprising a resinous substance and the fluid component of oxidized drying or semi-drying oil which is separated from a substantial proportion of unoxidized and non-hardening oil constituents of the oxidized oil, and is capable of hardening without further substantial oxidation, and sufficient solvent for said fluid component to maintain its fluidity. 10

20. A mouldable composition composed of 50% to 75% of filler material, a binder comprising that fluid component of oxidized drying or semi-drying oil which is capable of hardening without further substantial oxidation and is separated from a substantial proportion of unoxidized and non-hardening oil constituents of the oxidized oil, and sufficient solvent for said fluid component to maintain its fluidity. 15

21. Linoleum or similar composition composed of filler material and a binder comprising the hardened component of oxidized drying or semi-drying oil which, after oxidation of the oil is in fluid phase, is capable of hardening without further substantial oxidation, and has associated with it less than 6% of oil constituents soluble in petroleum ether. 25

22. Linoleum or similar composition composed of 50% to 75% of filler material and 25% to 50% of a binder comprising the hardened component of oxidized drying or semi-drying oil which, after oxidation of the oil is in fluid phase, is capable of hardening without further substantial oxidation, and which binder has associated with it less than 40 6% of unoxidized and non-hardening oil constituents of the oxidized oil soluble in petroleum ether. 35

23. The process which comprises the steps of subjecting a drying or semi-drying oil to an oxidizing treatment, discontinuing the oxidizing treatment prior to substantial coagulation of the oxidized oil, treating the products of oxidation to remove therefrom a substantial proportion of unoxidized oil constituents and non-hardening oil constituents, admixing filler material with the remaining fluid oxidized oil constituents to form a mouldable composition, treating the mixture to effect partial conversion of oxidized constituents therein into linoxyn, thereafter moulding the mix 55 by pressure, and subjecting the moulded mixture to treatment for converting oxidized oil constituents therein into linoxyn. 45

24. The process which comprises the steps of subjecting a drying or semi-drying oil to an oxidizing treatment, discontinuing the oxidizing treatment prior to substantial coagulation of the oxidized oil, treating the products of oxidation to remove therefrom a substantial proportion of unoxidized oil constituents and non-hardening oil constituents, admixing filler material with the remaining fluid oxidized oil constituents to form a mouldable composition, prolonging the mixing at elevated temperature, thereafter moulding the mix by pressure, and subjecting the moulded 70 mixture to treatment for converting oxidized oil constituents therein into linoxyn. 60